

Jan. 3, 1939.

J. D. PRICE

2,142,207

## FLOTATION PROCESS

Filed Oct. 29, 1935

2 Sheets-Sheet 1



INVENTOR.  
*JOHN D. PRICE*

BY

ATTORNEY.

Jan. 3, 1939.

J. D. PRICE

2,142,207

FLOTATION PROCESS

Filed Oct. 29, 1935

2 Sheets-Sheet 2



INVENTOR.  
JOHN D. PRICE

BY  
*J. D. Price*  
ATTORNEY.

## UNITED STATES PATENT OFFICE

2,142,207

## FLOTATION PROCESS

John D. Price, Pueblo, Colo., assignor, by mesne assignments, to The Colorado Fuel and Iron Corporation, a corporation of Colorado

Application October 29, 1935, Serial No. 47,251

26 Claims. (Cl. 209—165)

This invention relates to a flotation process and system of treating ores, and more particularly relates to a method and means for cleaning coal by flotation.

5 It is a principal object of the invention to create a value-carrying froth by a pressure control of the material being treated.

Another object of the invention is to eliminate violent agitation and the formation of eddy currents in the material in the froth-forming stages 10 of the treatment.

A further object of the invention is the creation of a froth of sufficient stability to promote good recovery during the flotation treatment, and of 15 sufficient brittleness to render the concentrate readily amenable to a subsequent dewatering treatment.

Still another object of the invention is the provision of a temperature control of the pressure 20 mediums employed in the process.

A still further object of the invention is to subject the material under treatment to a pulsating movement for accelerating the separation of values from gangue.

25 It is also an object of the invention to provide a process in which a comparatively small amount of reagent is employed as compared with the quantities required in other processes.

Other objects reside in novel details of construction and novel combinations and arrangements of parts as will more fully appear in the course of the following description.

Present froth flotation methods have proven advantageous in the concentration of minerals, 35 various metallic sulfides being particularly amenable to this treatment. In the froth flotation concentration of coal the same methods have been employed, generally with some variation in the reagent used to promote frothing and collection.

40 While satisfactory results may be attained by the foregoing methods insofar as the percentage of coal recovered is concerned, considerable difficulty is experienced in dewatering the concentrate, because of the stability of the froth; and 45 unless a stable froth is produced, the percentage of recovery is not high enough to warrant the expense of the treatment.

It has also been proposed to employ a separating vessel operated under partial vacuum for diffusing air throughout the pulp and thereby effecting a recovery of values. A high capacity vacuum pump is required and considerable difficulty is encountered due to leakage, and these conditions render the process expensive in operation.

The present invention permits the concentra-

tion of values in a froth of sufficient stability to insure high percentage recovery, but of sufficient brittleness to permit dewatering of the concentrate by inexpensive methods.

To produce a froth of this character, the pulp 5 under treatment in a confined state is subjected to pressure by the introduction of a gas under pressure into the pulp body, and subsequently, the pressure is released with the result that gas confined in the pulp body escapes, rising through 10 the same to its upper surface. This pressure release method of frothing effects a fine dispersion of gas throughout the pulp, subjecting the values to substantially constant association with bubbles of the gas until these values are carried 15 to the surface where they collect in a froth.

The velocity of the material under pressure is subject to control prior to the pressure release, and the rate at which the pressure is released is also controlled with the result that no violent agi- 20 tation occurs from this type of frothing.

The absence of violence in aerating the pulp permits use of froth of less stable character than would be necessary if violent agitation was used in order to effect a good recovery of values, and consequently smaller amounts of reagent are used 25 than in other processes.

Various gases may be employed for this purpose, such as air for example, but particularly effective results are attained when a gas containing a high percentage of  $\text{CO}_2$ , such as the gas evolved from a lime kiln, flue gas, or any other gas having a higher degree of solubility in water than air.

The reagent of the treatment may consist of 35 any of the soluble or insoluble materials commonly used for the flotation of coal, such as petroleum oils, coal tar oils, coal tar acids, etc.

In the co-pending application of Phillip M. Frantz, Serial No. 586,250, filed January 12, 1932 40 for Coal flotation process, reagents particularly well suited for coal flotation have been described, and may be effectively employed in the present invention. It is preferred that the reagent be introduced into the material being treated con- 45 tinuously in measured amounts.

It will be understood that the invention may be practiced in various types of apparatus, and to promote a better understanding of the various steps and treatments, the accompanying drawings 50 illustrate apparatus particularly effective in performing the process.

In the drawings, in the several views of which like parts have been similarly designated,

Figure 1 is a diagrammatic representation of

the assembly of elements employed in performing the process;

5 Figure 2 is a diagrammatic representation drawn to a reduced scale, of the application of temperature control means to apparatus for performing the process;

10 Figure 3 is a diagrammatic representation drawn to a reduced scale, of a modification of the reagent feed in the treatment; and

15 Figure 4 is a diagrammatic representation, also drawn to a reduced scale, of an assembly of elements for subjecting the ore or coal to successive treatments.

20 Referring now to Figure 1, the reference numeral 5 designates a conditioner for initially preparing the material for treatment. A suitable launder 6 or other means delivers pulp to the conditioner and a reagent feeder 7 is also provided for introducing reagent into the conditioner. The reagent feeder is preferably of the type which will deliver measured amounts of reagent.

25 The conditioner is provided with a discharge outlet 8, and agitators 9 in the conditioner thoroughly diffuse the reagent through the pulp prior to its discharge through outlet 8. In this connection, it is to be understood that any other suitable method of conditioning may be employed.

30 Material passing through outlet 8 is delivered into a collecting tank 10. The discharge from tank 10 is controlled by suitable means, such as a star feeder 12, and measured amounts of the conditioned pulp are introduced into a charging 35 vessel 13 by the star feeder 12.

35 The charging vessel 13 is provided with a suitable float-operated mechanism 14 for controlling a speed regulating mechanism 15, which in turn controls the operation of the star feeder 12. The 40 charging device 13 is also provided with a discharge outlet 16 controlled by an adjustable valve 17. The float-operated mechanism 14 functions to admit as much material into charger 13 as is being discharged out of the same, and in this way 45 the liquid level is maintained substantially constant.

50 The mechanism for controlling the outlet from charger 13 is represented as comprising a cone-valve 17 carried on a rack and pinion mechanism 18 operated by a hand wheel 19.

55 A pressure gas is supplied from a suitable source, such as a compressor (not shown) by valve-controlled pipes 20 and 21. Pipe 20 admits gas into the tank 13 at an elevation above its liquid level while pipe 21 extends into the tank 13 in the form of a perforated distributor 22, which admits the gas into the liquid body substantially uniformly throughout its cross-sectional area.

60 The pressure in the charger 13 above the liquid level is maintained substantially constant by means of an automatic pressure regulating device 23. It will be understood that the gas admitted above the liquid level should be proportioned to the gas admitted into the liquid, and where the pulp passing through outlet 16 is to be subjected to pressure changes of considerable magnitude, the pressure above the liquid body should be much in excess of the pressure within said body.

65 As an example, if gas from a compressor at twenty pounds per square inch pressure is introduced into the tank, effective results will be attained if said gas is maintained at fifteen 70 pounds pressure, above the liquid level.

75 The pulp, now more or less completely saturated with dissolved gas under pressure, is passed through outlet 16 into a conduit 24, which provides an unrestricted passage into a separator 25. At its discharge end 26, conduit 24 is of progressively increasing area, and the increase in area is in inverse ratio to the pressure of the pulp, which progressively approaches atmospheric pressure in its movement toward the discharge end of conduit 24.

10 The foregoing arrangement effects a velocity control of the pulp, the increased volume permitting sufficient expansion during pressure release to avoid undue turbulence and accelerated movement of the pulp.

15 The separator 25 is preferably open to the atmosphere at its upper end to provide a froth overflow 27, and if desired, a suitable froth crowder may be employed.

20 In Figure 1 the separator is illustrated as having its walls converging toward both ends from its mid-section, and the upper walls thereby function to squeeze the froth across the overflow 27. For convenience in illustration, the separator 25 is shown at substantially the same elevation 25 as the charger 13. In actual practice, it will generally be advantageous to position the separator at a higher elevation than the charger, the difference in elevation being dependent upon the pressure carried in the charger and varying directly 30 with the same. For this reason, the conduit 24 is broken in the drawings.

25 The discharge end of conduit 24 is preferably in the mid-section of separator 25 so that the upper portion of this tank constitutes the frothing zone 28. The part of the separator tank below the mid-section is a quiescent settling zone 29 through which the gangue material readily passes by gravity.

30 Inasmuch as certain values may be carried with the gangue toward the bottom of the tank, a second phase of aeration is provided in the quiescent zone. Air or other gas under pressure is admitted into the lower part of the tank through a distributor 30, preferably in the form of a series of tangential nozzles.

35 A whirling motion is imparted to the material in the lower portion of the tank 25, and any values which have descended from the upper frothing zone 28 are subjected to the buoyant influence of the gas and are carried up into the frothing zone and recovered in the froth.

40 Under certain conditions, it may be desirable to admit water instead of gas through distributor 30, as an example, to keep the settling material from becoming so thick that it will not flow readily.

45 A convenient arrangement for supplying gas to the distributor 30 is to have a conduit 31 connecting the upper side of star feeder 12 with distributor 30. Since the bottom of the star feeder 12 is exposed to the gas pressure in the upper portion of the charger 13, it follows that as the star revolves, (assuming a counter-clockwise motion), the bottom segment will carry with it a charge of gas at the pressure in the charger, which, if not released, will pass upward into collector 10, when such segment reaches the upper position, resulting in undesirable agitation in collector 10.

50 To avoid this, the inlet to conduit 31 is so arranged that when a gas-carrying segment of the feeder reaches an approximate horizontal position, the charge of gas which it carries will escape through the inlet into conduit 31.

As the gas discharge of star feeder 12 is intermittent, the gas supply to distributor 30 is also intermittent, creating a pulsating action in the separator 25 which facilitates separation of the values from the gangue and prevents accumulation of slimes on the separator walls. Return of liquid from separator tank 25 into conduit 31 during the intervals when no gas is flowing is prevented by a check valve 32 which may be of any suitable type.

Better results are attained in the frothing zone 28 when the liquid is in a state of comparative quiescence and to this end, swirl-restraining baffles 33, preferably in radial arrangement are provided in the mid-section of separator 25.

Gangue material settling by gravity in quiescent zone 29 passes into a sump 34 and is thereafter discharged by any suitable means, a star feeder 35 being illustrated as effective for this purpose.

While I do not wish to be limited to any particular driving assembly, a convenient arrangement has been illustrated in which a shaft 36 suitably journalled in conditioner 5 carries two pulleys 37 and 38 externally of conditioner 5, as well as the agitators 9 within the same. Pulley 37 is in driving connection with any suitable power source (not shown).

Pulley 38 is connected by a belt 39 with a pulley 40 on a shaft 41, which acts as the driving element of speed regulating mechanism 15. The star feeder 12 is in driving connection with mechanism 15 and its rate of rotation is controlled by the float mechanism 14, while the rate of rotation of star feeder 35 is varied in proportion to the quantity of gangue to be removed.

The operation will be described in connection with the separation of coal from rock and other material with which it occurs in nature, it being understood that the process is also adapted for the treatment of various types of mineralized matter.

The coal is first pulverized to a desired size by any well known method of comminution, for example, to a size which will permit all the pulverized material to pass through a screen of approximately ten meshes per inch.

Water is added as the material is fed into launder 6, or if wet grinding is employed, the water is added before grinding and the pulp is delivered to launder 6.

The coal in liquid suspension is thoroughly mixed in conditioner 5 with predetermined amounts of reagent. After the pulp is properly conditioned, it is passed into collecting tank 10.

The conditioned pulp is admitted from collector 10 into charger 13 by star feeder 12 operating under the control of mechanism 15, the quantity of pulp entering charger 13 being substantially the same as the discharge therefrom, to maintain the liquid level constant.

Pulp in charger 13 is subjected to pressure of a gas, lime kiln gas, for example, admitted simultaneously above and within the liquid body. The pressure of the gas is regulated so that the pressure above the liquid level exceeds the pressure of gas in the liquid body.

As a result of this condition, quantities of gas are absorbed and caused to go into solution in the liquid body. The gas pressure above the liquid level moves the pulp through discharge outlet 16 whenever valve 17 is opened, and the material under treatment thereupon moves freely through conduit 24 and discharges into separator 25.

It will be understood that once the desired liquid level has been attained and the gas pressures properly regulated, little, if any, regulation of valve 17 is required, and the operation thereafter is continuous, subject to a continuous feed.

As the pulp approaches the discharge end 26 of conduit 24, the pressure is progressively released, since separator 25 is maintained open to the atmosphere. The conduit 24 is of increasing cross-sectional area toward its discharge end 26 to accommodate the expansion of the pulp body occasioned by the pressure release.

Turbulence is avoided in this way and the gas which previously has been absorbed in the water, due to the high pressures, is liberated in the separator and rises to the surface in the form of minute bubbles. The coal particles are elevated by the bubbles and carried to the upper surface of the liquid body where they are collected in a froth and subsequently removed by overflow.

With each partial revolution of star feeder 12, gas under pressure is delivered to distributor 30 and a swirling motion is imparted to material in the lower portion 29 of the separator tank, and because of the intermittent admission of gas, a pulsating action is produced. Value settling with gangue are thereby floated and collected with the froth forming at the top of the liquid body.

From the foregoing it will be apparent that violent agitation is eliminated and as a result the froth required to collect the values does not have to be as stable as froth in devices employing violent agitation. Because of the extent of aeration induced by the pressure release, the values are continuously brought in contact with the bubbles rising to the surface. The two factors aforementioned, make possible an effective frothing even when comparatively small quantities of reagent are used.

The froth overflowing into a froth launder 42 on separator 25 is rather brittle and in proper condition for dewatering. Inexpensive dewatering methods may therefore be employed without loss of efficiency, and without special conditioning of the concentrate.

Certain modifications of the treatment hereinabove described have also been illustrated in the drawings. In Figure 2 a temperature control of the gases has been illustrated. This treatment is particularly effective where a flue gas is used in the process.

Water when cold will dissolve a larger amount of gas than when hot. For example, water at 10° C. will dissolve twice as much CO<sub>2</sub> as it will dissolve at 35° C. Hence, if the charger 13 is operated cold, and the pressure release takes place at a higher temperature, a greater evolution of gas will result, and an increased frothing action and separation will be attained.

The charger tank 13 illustrated in Figure 2 is similar in all respects to the charger tank 13 of Figure 1, except that constant pressure valves 43 on gas lines 20 and 21 are provided in place of the automatic regulating device 23.

Flue gas from a suitable source is delivered into a heat exchange device 44 through which the conduit 24 extends. The flue gas is cooled in the heat exchanger 44 and then passed on to a compressor 45, and thereafter the compressed gases are discharged into a storage tank 46, which communicates with pipes 20 and 21, for the supply of gas to tank 13.

The pulp under pressure passing through conduit 24 is heated as it passes through heat-exchanger 44, and upon discharging in separator

25, releases large quantities of gas which enhance the frothing action.

In the modification illustrated in Figure 3, preliminary conditioning of the pulp is eliminated, and the pulp is fed directly from launder 6 into collector 10. The charging in this device is identical with the charging illustrated in Figure 1. The absence of reagent from the pulp at this stage of the treatment avoids any preliminary frothing.

As the pulp passes through conduit 24, reagent is introduced therein by a pump 47 or other suitable feeding device, and due to the pressure in the material as it passes through conduit 24, 15 a thorough mixing of pulp and reagent is effected by the time the material is discharged into separator 25.

Whenever the discharge product passing through sump 34, contains considerable quantities 20 of valuable constituents, it may be desirable to re-treat this product and a convenient arrangement for so doing is illustrated in Figure 4.

The star feeder 35 controlling the discharge from sump 34, becomes the feeding device for a 25 second charger 13a and separator 25a, identical in all respects to those elements of the first treatment. Reagent is supplied through a feed pipe 48 before the material reaches the star feeder 35.

In the various modifications, a discharge outlet 30 49 of the valve-controlled type can be provided in the bottom of conduit 24, to permit cleaning of the same.

From the foregoing it is apparent that the 35 process may be conveniently practiced in apparatus of a different character than that indicated in the drawings. It is likewise apparent that the methods hereinabove described may be employed in treating various different kinds of solid material in liquid suspension.

40 Changes and modifications in the various steps and treatments, and arrangement of parts may be availed of within the spirit and scope of the invention as defined in the hereunto appended claims.

45 What I claim and desire to secure by Letters Patent is:

1. The process of treating solids in liquid suspension, comprising, confining a body of solids in liquid suspension, introducing gas under pressure 50 into said body beneath the surface thereof, subjecting the body to the action of a pressure gas externally applied, while so confined, and inducing a separation of constituent materials in the body by progressively decreasing pressure on the body until it reaches atmospheric pressure, in a releasing action.

2. The process of treating solids in liquid suspension, comprising, confining a body of solids in liquid suspension, introducing gas under pressure 60 into said body beneath the surface thereof, subjecting the body to the action of a pressure gas externally applied, while so confined, and inducing a separation of constituent materials in the body by exposing the body to the atmosphere in a movement at a progressively reduced velocity.

3. The process of treating solids in liquid suspension, comprising, confining a body of solids in liquid suspension, simultaneously introducing gas under pressure into said body beneath the surface 70 thereof and externally of the same while so confined, to thereby subject the body to compression, and inducing a separation of constituent materials in the body by a subsequent release of pressure on the body in a movement at a progressively reduced velocity.

4. The process of treating solids in liquid suspension, comprising, confining a body of solids in liquid suspension, simultaneously introducing gas under pressure into said body beneath the surface thereof and externally of the same while so confined, the pressure of the gas externally of the body being in excess of the pressure of the gas within the same, to thereby subject the body to compression, and inducing a separation of constituent materials in the body by a subsequent release of pressure on the body. 10

5. In a froth flotation process, the steps of simultaneously cooling a pressure gas being introduced into a pulp under treatment, and heating the pulp in which the gas has previously been 15 introduced after compression by utilizing heat withdrawn from the cooled gases as the heating medium.

6. The process of coal flotation comprising, mixing a coal-containing pulp with a flotation agent, subjecting the mixture to compression while introducing a gas under pressure therein beneath its surface, and floating the coal constituents of the mixture in a froth formed by release of the pressure on the mixture. 20

7. The process of coal flotation comprising, mixing a coal-containing pulp with a flotation agent, subjecting the mixture to compression while entering a soluble gas under pressure into solution beneath its surface, and floating the coal constituents of the mixture in a froth formed by release of the pressure on the mixture. 25

8. The process of coal flotation comprising, subjecting a coal-containing pulp to compression while introducing a gas under pressure therein beneath its surface, introducing a flotation agent into the compressed pulp, moving the pulp through a zone of decreasing pressure, and floating the coal constituents of the mixture in a froth formed by release of the pressure on the pulp. 30

9. In a process of treating solids in liquid suspension, including the treatment of material in intercommunicating aerating and settling zones, the steps of continuously subjecting solids in liquid suspension to the action of an expanding body 45 of gas in the aerating zone, and intermittently subjecting material in the settling zone to the action of an expanding body of gas.

10. The froth flotation process comprising charging a pulp with a compressible fluid, compressing the charged pulp, inducing a flow of the pulp to a zone of progressively decreasing pressure, progressively expanding the volume of the pulp in its passage through said zone, discharging the pulp from said zone at approximately atmospheric pressure to induce frothing in the pulp, and maintaining a quiescent zone in the discharged body below the zone of frothing for gravity settling of material not acted on by the frothing. 50

11. The froth flotation process comprising charging a pulp with a compressible fluid, compressing the charged pulp, inducing a flow of the pulp and a flotation agent to a zone of progressively decreasing pressure, progressively expanding the volume of the pulp in its passage through said zone, discharging the pulp from said zone at approximately atmospheric pressure to induce frothing in the pulp, and maintaining a quiescent zone in the discharged body below the zone of frothing for gravity settling of material not acted on by the frothing. 55

12. The froth flotation process comprising charging a pulp with a compressible fluid, compressing the charged pulp, inducing a flow of the 70 pulp and a flotation agent to a zone of progressively decreasing pressure, progressively expanding the volume of the pulp in its passage through said zone, discharging the pulp from said zone at approximately atmospheric pressure to induce frothing in the pulp, and maintaining a quiescent zone in the discharged body below the zone of frothing for gravity settling of material not acted on by the frothing. 75

pulp and a flotation agent to a zone of progressively decreasing pressure, progressively increasing the volume of the pulp in its passage through said zone, discharging the pulp from said zone at an elevated point at approximately atmospheric pressure to induce frothing in the pulp, subjecting the discharge pulp to a pulsating action to promote separation, overflowing a concentrate collected in the froth at an elevated point of discharge, and removing gangue from the pulp by gravity settling below the zone of frothing.

13. A system of treating solids in liquid suspension, comprising a charging vessel, means for intermittently feeding measured amounts of solids in liquid suspension to said vessel, means for admitting a pressure fluid into said vessel for charging and compressing material fed into the same, an open separating vessel having an elevated overflow and a discharge for settled material, means for delivering the charged material from the charging vessel into the separating vessel above its discharge, and at substantially atmospheric pressure to induce aeration by release of pressure on the material, a conduit to receive gas escaping from the charging vessel during each delivery of feed thereto, and a discharge nozzle disposed in the lower portion of the separating vessel in operative connection with the conduit for effecting a pulsating movement of the material settling by gravity in said vessel.

14. A system of treating solids in liquid suspension, comprising a charging vessel, means for intermittently feeding measured amounts of solids in liquid suspension to said vessel, means for admitting a pressure fluid into said vessel for charging and compressing material fed into the same, an open separating vessel having an elevated overflow and a discharge for settled material, means for delivering the charged material from the charging vessel into the separating vessel above its discharge, and at substantially atmospheric pressure to induce aeration by release of pressure on the material, a conduit to receive gas escaping from the charging vessel during each delivery of feed thereto, a discharge nozzle disposed in the lower portion of the separating vessel in operative connection with the conduit for effecting a pulsating movement of the material settling by gravity in said vessel, and a valve in the conduit for preventing the escape of liquid through the nozzle when gas is not flowing through the conduit.

15. Froth flotation apparatus, comprising a charging vessel having a feed inlet and a discharge outlet, a valve controlling the rate of discharge thru said outlet, a mechanism controlled by the pulp level in the charging vessel for regulation of the rate of pulp feed, means for introducing a pressure gas into the pulp body in the charging vessel, means for introducing gas under pressure into the charging vessel above the liquid level, and a separator chamber in communication with the discharge.

16. Froth flotation apparatus, comprising a charging vessel having a feed inlet and a discharge outlet, a valve controlling the rate of discharge thru said outlet, a mechanism controlled by the pulp level in the charging vessel for regulation of the rate of pulp feed, an element for introducing a pressure gas into the charging vessel above and below the liquid level, and a separator chamber in communication with the discharge.

17. A system of treating solids in liquid suspension, comprising a charging vessel having a controlled discharge determining a liquid level there-

in, means for feeding measured amounts of solids in liquid suspension to said vessel, means for admitting a pressure fluid into said vessel beneath the liquid level for charging and compressing material fed into the same, a separating vessel communicating with the atmosphere and having an overflow at a higher elevation than the liquid level in the charging vessel and having a discharge for settled material therebelow, and means for delivering the charged material from the charging vessel into the separating vessel above its discharge, in a continuous operation and at substantially atmospheric pressure to induce aeration by release of pressure on the material.

18. The improvement in a froth flotation process in which a pulp and a gas are subjected to superatmospheric pressure in one zone and is then discharged into a frothing zone maintained at atmospheric pressure, to induce frothing, which comprises discharging a pulp body subjected to such superatmospheric pressure, into a zone of frothing through a restricted zone of progressively increasing area in a movement of progressively decreasing velocity.

19. The improvement in a froth flotation process in which a pulp and a gas are subjected to superatmospheric pressure in one zone and is then discharged into a frothing zone maintained at atmospheric pressure, to induce frothing, which comprises discharging a pulp body subjected to such superatmospheric pressure, into a zone of frothing through a zone in which the pressure on the body progressively approaches atmospheric in a movement of progressively decreasing velocity.

20. In a froth flotation process, the steps of compressing a confined body of pulp by simultaneously introducing a gas under pressure into the body of pulp beneath its surface and exteriorly of the same within the zone of confinement, and discharging the compressed body into a frothing zone through a restricted zone of progressively increasing area, in a movement in which the pressure on the body progressively approaches atmospheric.

21. In a froth flotation process, the steps in a continuous operation, of compressing a pulp body, while subjected to a restricted flow, by simultaneously introducing a gas under pressure into the pulp body beneath its surface and exteriorly of the same within the restricted zone, and continuously discharging compressed pulp from the restricted zone into a frothing zone in a movement at a progressively decreasing velocity, and in which pressure on the moving pulp immediately prior to its entrance into the frothing zone is substantially equal to atmospheric pressure.

22. The froth flotation process which comprises introducing a water-soluble gas into a confined body of pulp, compressing the pulp containing the gas, maintaining a predetermined pulp temperature during compression at which the gas readily enters into solution, moving the compressed pulp to a discharge in a pressure-release zone, and subjecting the moving pulp to a heating action.

23. The froth flotation process which comprises introducing a gas containing carbon dioxide into a confined body of pulp, compressing the pulp containing the gas, maintaining a predetermined pulp temperature during compression at which the gas readily enters into solution, moving the compressed pulp to a discharge in

5

10

15

20

25

30

35

40

45

50

55

60

65

70

75

a pressure-release zone, and subjecting the moving pulp to a heating action.

24. The froth flotation process which comprises introducing a water-soluble gas into a confined body of pulp, compressing the pulp containing the gas, maintaining a predetermined pulp temperature during compression at which the gas readily enters into solution, moving the compressed pulp to a discharge in a pressure-release zone, and subjecting the moving pulp to a heating action effective for accelerating evolution of gas in the discharging pulp.

25. The process of coal flotation which comprises, mixing a coal-containing pulp with a flotation agent, introducing a soluble gas into the

pulp beneath its surface, subjecting the pulp to treated to compression, and then floating coal constituents of the pulp by discharging the compressed pulp into a frothing zone maintained at atmospheric pressure, in a movement of progressively decreasing velocity.

26. In a froth flotation process, the step of preparing pulp for a frothing action by simultaneously introducing gas under pressure exteriorly of a confined body of pulp and entering such gas into solution in the pulp while maintaining a pressure exteriorly of the body in excess of the pressure within the same, during such gas-introducing action.

JOHN D. PRICE. 15